

# UNITED STATES PATENT OFFICE.

WILLIAM H. GOODENOUGH, OF CAMPAS, WASHINGTON.

## PROCESS OF MAKING PAPER.

1,257,996.

Specification of Letters Patent. Patented Mar. 5, 1918.

No Drawing.

Application filed August 29, 1917. Serial No. 188,791.

*To all whom it may concern:*

Be it known that I, WILLIAM H. GOODENOUGH, a citizen of the United States, residing at Camas, in the county of Clark 5 and State of Washington, have invented new and useful Improvements in Processes of Making Paper, of which the following is a specification.

This invention relates to a method 10 wherein an alkali is introduced into the paper making stock and has for its object to make the stuff run better on the machine, screening much more freely and causing less "breaks" as the web goes through the 15 presses; also to render the sheet capable of taking a superior finish. It avoids the use of all size. It relates particularly to newsprint paper, the finished product taking cuts and prints much better than a sheet whose 20 fibers have not been so treated.

In the process of making newsprint paper, the ground wood stock and the sulfite stock are usually mixed in the proper proportions and beaten in a beater engine and 25 it is at this point in the paper-making process that I introduce two pounds of sal-soda into approximately fifteen hundred pounds of paper stock thus mixing it intimately with the paper making fibers. In 30 mills which use the "tank system" and have discarded the beaters, the proper amount of sal-soda can be added in the "mixing tanks" whose agitators will diffuse the soda throughout the stuff. While I have attained 35 the best results with sal-soda and prefer to use sodium in that form, yet soda-ash, caustic soda and the like can be used with satisfactory results.

It is a source of constant trouble on the 40 screens of a paper machine that strings of pulp fiber form which work into the pulp stock and cause lumps which result in frequent breaking of the tender web of paper as it goes through the presses of the ma-

chine. I have discovered that fibers treated 45 with an alkali as above set forth, will go through the screens much more freely and with much less tendency to form "strings," so that "breaks" from this cause on the paper machine are reduced to a minimum 50 and the output of the machine increased. Also the "felting" quality of the fibers is improved, forming a closer sheet, which takes an improved finish from the calendering. The improvement in finish is marked 55 and the usual sizing may be omitted, effecting a reduction of cost. When the ground wood or the sulfite stock has rosin or pitch in it the sodium acts as a corrective and trouble from this source is avoided. 60

I claim,—

1. In the process of making news-print paper the addition of two pounds of sal-soda to fifteen hundred pounds of paper stock. 65
2. In the process of making news-print paper the addition in the beater engine of approximately two pounds of sal-soda to approximately fifteen hundred pounds of paper stock. 70
3. In the process of making newsprint paper the addition in the mixing tank of approximately two pounds of sal-soda to approximately every fifteen hundred pounds of paper stock. 75
4. In the process of making newsprint paper the addition of approximately two pounds of an alkali to approximately every fifteen hundred pounds of paper stock. 80
5. Paper impregnated with an alkali, 85 there being about .0013½% of said alkali added to the paper material during the process of manufacture.
6. In the process of making newsprint paper the addition of an alkali to the paper stock. 85

W. H. GOODENOUGH.